

Patented Jan. 15, 1946

2,393,008

# UNITED STATES PATENT OFFICE

2,393,008

## ORE CONCENTRATION

Herbert S. Woodward and William A. Bates,  
Gabbs, Nev., assignors, by mesne assignments,  
to Defense Plant Corporation, Washington,  
D. C.

No Drawing. Application May 9, 1944,  
Serial No. 534,811

12 Claims. (Cl. 209—166)

This invention relates to the beneficiation of magnesium-bearing ores, especially magnesite, and has for its object the separation of magnesite from its accompanying impurities in the ore by froth flotation. More particularly, the invention provides an improved method of separating siliceous materials from magnesite by froth flotation in an economical and efficient operation.

Magnesites occurring in nature commonly have associated with them objectionable quantities of siliceous impurities, such as talcs and serpentines. Such impurities reduce the value of the ore, or limit its usage, for the manufacture of magnesium metal and refractory materials. In the beneficiation of magnesite, it is customary selectively to mine and sort or screen the ore to eliminate the low-grade material and associated gangue. Several froth flotation processes have been proposed for concentrating magnesite ores, involving the use of cationic collectors and methyl amyl alcohol to float the siliceous impurities, and the use of naphthenic acids for floating magnesite, utilizing other reagents to depress the siliceous and calcareous components. The flotation of a talc concentrate from magnesite-containing gangue, using a wetting agent involving sodium or ammonium alkyl sulphates, has been suggested. Due to the well-known floatability of the associated silica minerals, the direct flotation of magnesite from these impurities has failed to yield a product of sufficient purity for many industrial uses.

The proposed practices of floating the silicate impurities away from the magnesite either leave an undesirable amount of the silicate minerals with the residual magnesite fraction, or, in an attempt to obtain a magnesite fraction of low silica content, remove an undesirably large amount of the magnesite along with the siliceous froth, with resultant lower recoveries of magnesite and high operating cost. These proposed practices fail to recover a high magnesia product low in silica from ores containing in the neighborhood of 5% or more of acid insoluble material, and, for the most part, have the economic disadvantage that they require relatively large quantities of expensive reagents and, in many instances, require the preliminary removal of slimes in order to obtain a high-grade product and to reduce the reagent consumption to a practical basis. The removal of slimes further lowers the recovery and increases the cost of the recovered magnesite.

It is an object of this invention to overcome the disadvantages of the practices proposed heretofore and to provide an improved method for the economical separation by froth flotation of a magnesite product low in silica.

Based upon our discoveries, the invention provides an improved method of separating a rela-

tively pure magnesite from ore containing siliceous impurities by froth flotation, involving the incorporation in a pulp of the ore a reagent comprising saturated aliphatic monocarboxylic acids, the esters of such acids, or mixtures of such acids and esters for the floating of siliceous impurities.

The invention is advantageously applicable to the treatment of low-grade magnesite ores which are difficult to handle by present flotation procedure. An example of such ores is the large, massive magnesite deposits located in northern Nye County, Nevada. Such ores contain variable proportions of siliceous impurities, including talcs, serpentines and fosterites. These magnesite ores may have associated magnesium minerals, such as brucite and hydromagnesite, and in places may have undesirably large amounts of "R<sub>2</sub>O<sub>3</sub>" contaminants. While some of the siliceous and other impurities are present in relatively coarse aggregates, it is usually necessary to grind the ore to suitable fineness, for example, to approximately minus 100 mesh, to free the impurities from the associated magnesite.

In practicing the invention, the ore is first ground to a suitable degree of fineness and the ore, either during or after grinding, is mixed with water to form a free-flowing pulp. The ore is preferably comminuted by wet grinding in a closed circuit with a classifier. The flotation reagents may be introduced into the grinding circuit, or they may be added in a separate conditioning treatment between the grinding and flotation circuits. Alternatively, the reagents may be added immediately ahead of the flotation circuit. In using a collector reagent in accordance with the invention, we may use mixed aliphatic acids obtained from petroleum, and preferably having a boiling range between 160° and 250° C. Such aliphatic acids are especially desirable from a standpoint of cost and their effective selective action in the floating of siliceous impurities. We may also use very effectively saturated aliphatic monocarboxylic acids containing from 4 to 9 carbon atoms, such as butyric and ethyl caproic acids, as reagents. Alternatively, esters made by reacting saturated aliphatic monocarboxylic acids having from 4 to 9 carbon atoms with saturated aliphatic alcohols may be used as reagents. Examples of such esters are methyl amyl butyrate, ethyl hexyl butyrate and the methyl isobutyl ester of 2-ethyl caproic acids. As a collector reagent we may also use mixtures of such aliphatic acids obtained from petroleum, saturated aliphatic monocarboxylic acids, and esters made by reacting saturated aliphatic monocarboxylic acids having from 4 to 9 carbon atoms with saturated aliphatic alcohols. An example of such a mixture consists of 75% mixed aliphatic acids obtained from petroleum and 25% of 2-ethyl caproic acid. The esters formed by react-

ing saturated aliphatic monocarboxylic acids having from 4 to 9 carbon atoms with saturated aliphatic monohydric alcohols, including primary, secondary and tertiary alcohols are desirable reagents or constituents of reagent mixtures.

These reagents of the invention are normally added ahead of the flotation circuit. Conjointly with, or preferably following the introduction of the collector reagent, the pulp is subjected to aeration, usually accompanied by mechanical agitation in any suitable flotation cell or series of cells, and the siliceous impurities are selectively carried to the surface in a froth, where they may be removed. The residual magnesite pulp, substantially impoverished in siliceous impurities, may be dewatered and used as a source of magnesia for the production of magnesium metal or magnesia refractories, or other magnesian products requiring a low-silica material or the residual magnesite pulp may be treated by flotation or chemical processes further to remove associated siliceous and calcareous impurities from the magnesite product. For example, the residual magnesite pulp may be subjected to a second froth flotation treatment for selectively floating of the magnesite which is removed as a froth. The magnesite thus impoverished in calcareous contaminants is removed from the operation, dewatered and used as a source of magnesia in the production of magnesium or magnesian products.

In the following illustrative examples of the present invention, magnesite ore from Nye County, Nevada, was used.

#### Example I

The ore was crushed and wet-ground in a closed circuit with a classifier so that approximately all the ore passed a 100-mesh sieve. The resulting pulp, comprising approximately one part of ore to four parts of water, was conditioned with approximately 0.3 pound of a mixture of 75% mixed aliphatic acids obtained from petroleum and 25% of 2-ethyl caproic acid per ton of ore. The pulp was then subjected to froth flotation and the following products were obtained:

| Product             | Percent of feed | Analysis, percent |                               |      |
|---------------------|-----------------|-------------------|-------------------------------|------|
|                     |                 | Acid insoluble    | R <sub>2</sub> O <sub>3</sub> | CaO  |
| Feed                | 100.0           | 5.45              | 2.28                          | 9.40 |
| Froth concentrate   | 11.90           | 35.46             | 2.17                          | 7.47 |
| Tailing (magnesite) | 88.10           | 1.41              | 2.29                          | 9.66 |

The magnesite enriched tailing was then subjected to a further flotation treatment. The magnesite was selectively floated in this operation and taken off as a rougher concentrate, which was recleaned. The results of this test are shown below:

| Product             | Percent of original feed | Analysis, percent |                               |       |
|---------------------|--------------------------|-------------------|-------------------------------|-------|
|                     |                          | Acid insoluble    | R <sub>2</sub> O <sub>3</sub> | CaO   |
| Cleaner concentrate | 58.6                     | 0.42              | 0.60                          | 6.77  |
| Cleaner tailing     | 17.1                     | 1.75              | 2.05                          | 14.84 |
| Rougher concentrate | 75.7                     | 0.72              | 0.93                          | 8.60  |
| Rougher tailing     | 12.4                     | 5.60              | 10.67                         | 16.23 |

#### Example II

Magnesite pulp ground to pass approximately 100-mesh sieve was conditioned with approxi-

mately 0.3 pound of mixed aliphatic acids obtained from petroleum per ton of ore. The conditioned pulp was subjected to froth flotation and the following products were obtained:

| Product             | Percent of feed | Analysis, percent |                               |       |
|---------------------|-----------------|-------------------|-------------------------------|-------|
|                     |                 | Acid insoluble    | R <sub>2</sub> O <sub>3</sub> | CaO   |
| Feed                | 100.0           | 5.54              | 2.19                          | 10.00 |
| Froth concentrate   | 9.10            | 45.17             | 1.72                          | 6.50  |
| Tailing (magnesite) | 90.9            | 1.57              | 2.23                          | 10.35 |

The magnesite tailing resulting from this flotation step was subjected to an additional flotation treatment to reduce the lime content of the magnesite. A rougher concentrate was floated and recleaned. The results of the second flotation were as follows:

| Product             | Percent of original feed | Analysis, percent |                               |       |
|---------------------|--------------------------|-------------------|-------------------------------|-------|
|                     |                          | Acid insoluble    | R <sub>2</sub> O <sub>3</sub> | CaO   |
| Cleaner concentrate | 64.50                    | 0.50              | 0.63                          | 7.50  |
| Cleaner tailing     | 12.4                     | 2.67              | 2.77                          | 16.30 |
| Rough concentrate   | 77.0                     | 0.85              | 0.97                          | 9.32  |
| Rougher tailing     | 13.9                     | 5.61              | 9.75                          | 16.00 |

#### Example III

Wet-ground magnesite pulp passing approximately 100-mesh sieve was conditioned with approximately 0.3 pound per ton of methyl amyl butyrate and a siliceous froth was removed. The results of this test were as follows:

| Product             | Percent of feed | Analysis, percent |                               |       |
|---------------------|-----------------|-------------------|-------------------------------|-------|
|                     |                 | Acid insoluble    | R <sub>2</sub> O <sub>3</sub> | CaO   |
| Feed                | 100.0           | 5.50              | 3.07                          | 9.75  |
| Froth concentrate   | 6.76            | 57.88             | 1.20                          | 4.90  |
| Tailing (magnesite) | 93.24           | 1.63              | 2.47                          | 10.10 |

The tailing from this test was subjected to a second froth flotation treatment wherein the magnesite fraction was floated and the calcareous material was depressed.

#### Example IV

The magnesite pulp, wet-ground to pass approximately 100-mesh sieve, was conditioned with 0.3 pound of butyric acid per ton of ore and with 0.15 pound pine oil per ton of ore. The insoluble impurities were collected in a froth concentrate with the following results:

| Product             | Percent of feed | Analysis, percent |                               |      |
|---------------------|-----------------|-------------------|-------------------------------|------|
|                     |                 | Acid insoluble    | R <sub>2</sub> O <sub>3</sub> | CaO  |
| Feed                | 100.0           | 5.44              | 2.25                          | 9.60 |
| Froth concentrate   | 8.35            | 49.01             | 1.81                          | 6.10 |
| Tailing (magnesite) | 91.65           | 1.57              | 2.30                          | 9.92 |

The low-silica, magnesite-enriched tailing resulting from this test was given a further flotation treatment wherein low-silica, low-lime magnesite froth was produced.

While 0.3 pound of reagent per ton of magnesite ore treated was used in the foregoing specific examples, the quantity of mixed aliphatic acids obtained from petroleum, saturated aliphatic monocarboxylic acids having from 4 to 9 carbon

atoms, esters made by reacting saturated aliphatic monocarboxylic acids having from 4 to 9 carbon atoms with saturated aliphatic alcohols, and mixtures of such mixed aliphatic acids obtained from petroleum, saturated aliphatic monocarboxylic acids having from 4 to 9 carbon atoms and esters made by reacting saturated aliphatic monocarboxylic acids having from 4 to 9 carbon atoms with saturated aliphatic alcohols and any other desired quantities of these reagents may be used in treating such ores depending upon the conditions of treatment and the results sought. The particular quantity of reagent will depend upon such factors as the character of the ore, the physical characteristics of the pulp, the degree of conditioning used and the quality of the reagent employed. The magnesite product resulting from the first flotation step may be further beneficiated by calcining the magnesite and removing the lime by chemical methods.

We claim:

1. In the froth flotation separation of magnesite from siliceous impurities contained in ore, the improved method which comprises incorporating in a pulp of the ore a collector reagent comprising mixed aliphatic acids obtained from petroleum and having a boiling range of from 160° to 250° C., subjecting the pulp to a flotation treatment and selectively separating siliceous impurities as a froth from the magnesite.

2. In the froth flotation separation of magnesite from siliceous impurities contained in ore, the improved method which comprises incorporating in a pulp of the ore a collector reagent comprising a saturated monocarboxylic aliphatic acid having from 4 to 9 carbon atoms, subjecting the pulp to a flotation treatment and selectively separating siliceous impurities as a froth from the magnesite.

3. In the froth flotation separation of magnesite from siliceous impurities contained in ore, the improved method which comprises incorporating in a pulp of the ore a collector reagent comprising an ester formed by reacting a saturated aliphatic monocarboxylic acid having from 4 to 9 carbon atoms with a saturated aliphatic alcohol, subjecting the pulp to a flotation treatment and selectively separating siliceous impurities as a froth from the magnesite.

4. In the froth flotation separation of magnesite from siliceous impurities contained in ore, the improved method which comprises incorporating in a pulp of the ore a collector reagent comprising a mixture of saturated aliphatic acids obtained from petroleum, and an ester formed by reacting saturated aliphatic monocarboxylic acid having from 4 to 9 carbon atoms with a saturated aliphatic alcohol, subjecting the pulp to a flotation treatment and selectively separating siliceous impurities as a froth from the magnesite.

5. In the froth flotation separation of magnesite from siliceous impurities contained in ore, the improved method which comprises incorporating in a pulp of the ore a collector reagent comprising butyric acid, subjecting the pulp to a flotation treatment and selectively separating siliceous impurities as a froth from the magnesite.

6. In the froth flotation separation of mag-

nesite from siliceous impurities contained in ore, the improved method which comprises incorporating in a pulp of the ore a collector reagent comprising methyl amyl butyrate, subjecting the pulp to a flotation treatment and selectively separating siliceous impurities as a froth from the magnesite.

7. In the froth flotation separation of magnesite from siliceous and calcareous impurities contained in ore, the improved method which comprises incorporating in a pulp of the ore a collector reagent comprising a saturated monocarboxylic aliphatic acid having from 4 to 9 carbon atoms, and subjecting the pulp to a flotation treatment and selectively separating siliceous impurities as a froth from the magnesite.

8. In the froth flotation separation of magnesite from siliceous impurities contained in ore, the improved method which comprises incorporating in a pulp of the ore a collector reagent comprising an ester formed by reacting a saturated aliphatic monocarboxylic acid having from 4 to 9 carbon atoms with a saturated aliphatic monohydric alcohol, subjecting the pulp to a flotation treatment and selectively separating siliceous impurities as a froth from the magnesite.

9. In a froth flotation separation of magnesite from siliceous impurities contained in ore, the improved method which comprises incorporating in a pulp of the ore a collector reagent comprising an ester formed by reacting a saturated aliphatic monocarboxylic acid having from 4 to 9 carbon atoms with a saturated aliphatic primary monohydric alcohol, subjecting the pulp to a flotation treatment and selectively separating siliceous impurities as a froth from the magnesite.

10. In the froth flotation separation of magnesite from siliceous impurities contained in ore, the improved method which comprises incorporating in a pulp of the ore a collector reagent comprising a mixture of saturated aliphatic acids obtained from petroleum and an ester formed by reacting saturated aliphatic monocarboxylic acid having from 4 to 9 carbon atoms with a saturated aliphatic monohydric alcohol, subjecting the pulp to a flotation treatment and selectively separating siliceous impurities as a froth from the magnesite.

11. In the froth flotation separation of magnesite from siliceous impurities contained in ore, the improved method which comprises incorporating in a pulp of the ore a collector reagent comprising a mixture of saturated aliphatic acids obtained from petroleum and an ester formed by reacting saturated aliphatic monocarboxylic acid having from 4 to 9 carbon atoms with a saturated aliphatic primary monohydric alcohol, subjecting the pulp to a flotation treatment and selectively separating siliceous impurities as a froth from the magnesite.

12. In the froth flotation separation of magnesite from siliceous impurities contained in ore, in which pine oil is used as a frothing agent, the improved method which comprises incorporating in a pulp of the ore a collector reagent comprising butyric acid, subjecting the pulp to a flotation treatment and selectively separating siliceous impurities as a froth from the magnesite.

HERBERT S. WOODWARD.  
WILLIAM A. BATES.